

## UNITED STATES PATENT OFFICE.

JOSEPH SEYER, OF HAWTHORNE, NEW JERSEY, ASSIGNOR TO STANDARD SILK DYE-  
ING CO., A CORPORATION OF NEW JERSEY.

## PROCESS OF DYEING SILK.

No Drawing.

Application filed March 15, 1923. Serial No. 625,257.

*To all whom it may concern:*

Be it known that I, JOSEPH SEYER, a citizen of the United States, a resident of Hawthorne, in the county of Passaic and State 5 of New Jersey, have invented a certain new and useful Process of Dyeing Silk, of which the following is a specification.

This invention relates to a process of dyeing silk, and more particularly to a process 10 of dyeing weighted silk with a direct dye.

It is an object of this invention to dye silk of various kinds by avoiding the use of acid liquids, which have an injurious effect upon certain forms of silk such as tin 15 weighted silks. It is a further object of the invention to dye silk of various kinds in various shades and colors by the use of direct dyes in non-acid media or dye liquors. Further objects of the invention will appear 20 hereinafter.

In the preferred embodiment of the invention the following process is employed:

Silk is tin weighted in the usual manner, while in the form of skeins or threads, and 25 it is then treated in a weak alkaline bath with a direct dye to produce any desired color or shade thereof. For the bath material di-sodium hydrogen phosphate is dissolved in water in the proportion of 5 lbs. 30  $Na_2HPO_4$  in 250 gallons of water. The solution is free of acids.

Silk, either in the form of a skein or piece goods, is dyed in the above described liquor with the aid of a direct dye. The process 35 is applied with great advantage in the case of silks that have been previously weighted, either in the form of a skein or in the form of piece goods. The absence of acid in the liquid prevents injurious action in connection with the tin salt, and the presence of the di-sodium hydrogen phosphate facilitates the production of an even color.

The process can be economically carried out and without risk of seriously injuring 40 the goods. The operation is simple and is of general application. The process may

also be carried out in connection with the process described in the Cole Patent, 1,446,834, in which is described a process of weighting silk before throwing it, or before weaving it. Thus the dyeing step which constitutes the final step, in one embodiment of the Cole process, may be carried out as above described with the aid of a direct dye. 55

As many apparently widely different embodiments of this invention may be made without departing from the spirit thereof, it is to be understood that I do not limit myself to the preferred embodiments described except as indicated in the following claims. 60

I claim:

1. The process of dyeing silk piece goods comprising treating them with a weak alkaline solution containing a direct dye. 65

2. The process of dyeing weighted silk piece goods comprising treating them with a weak alkaline solution containing a direct dye. 70

3. The process of dyeing silk piece goods weighted in the skein comprising treating them with a weak alkaline solution containing a direct dye. 75

4. The process of dyeing silk piece goods weighted in the skein comprising treating them with a di-sodium hydrogen phosphate solution containing a direct dye. 80

5. The process of dyeing silk piece goods weighted with a tin compound which comprises treating them with di-sodium phosphate solution containing a direct dye. 85

6. The process of dyeing silk piece goods weighted in the skein with a tin compound, which comprises treating them with di-sodium phosphate solution containing a direct dye. 90

In testimony that I claim the foregoing, I have hereunto set my hand this 14th day of March, 1923.

JOSEPH SEYER.